

# UNITED STATES PATENT OFFICE.

MARCELLO VON PIRANI, OF WILMERSDORF, NEAR BERLIN, GERMANY, ASSIGNOR TO  
GENERAL ELECTRIC COMPANY, A CORPORATION OF NEW YORK.

## METHOD OF PREFORMING REFRACATORY MATERIAL PRIOR TO ROLLING.

1,093,203.

Specification of Letters Patent. Patented Apr. 14, 1914.

No Drawing.

Application filed November 23, 1912. Serial No. 733,077.

To all whom it may concern:

Be it known that I, MARCELLO VON PIRANI, a citizen of the Italian Kingdom, residing at Wilmersdorf, near Berlin, Germany, have 5 invented certain new and useful Improvements in the Method of Preforming Refractory Material Prior to Rolling, of which the following is a specification.

In the rolling of refractory metals such 10 as tungsten, which have a certain amount of brittleness, difficulties arise due to the development of cracks or fractures. These cracks are caused by the radical changes of form to which the material is subjected, and 15 the greater the changes of form the more cracked the material becomes. The changes of form are greatest at the beginning of the rolling operation and therefore the danger of cracking is greatest at this time.

20 Metals which are in general more or less easy to work show a tendency to a certain degree to crack on being rolled, but these difficulties may be met by giving to these metals before they come between the rollers, 25 a cross-section by hammering, forging or the like which nearly corresponds to the cross-section when rolled. Thereby the changes of form in rolling are greatly reduced. Such manipulation, however, cannot be ef- 30 fected with refractory, brittle metals, since, as is well known, they are not workable in this sense under ordinary conditions.

The object of this invention is to render 35 these metals workable and it is accomplished by giving to the material to be rolled a form which is similar to the cross-section which it is to have after being rolled. It might at first be thought that one way of 40 doing this would be by casting it in molds in this cross-sectional form. Practically, however, casting in proper cross-section is not feasible on account of the extraordi- narily high fusing temperatures of the ma- 45 terials and the difficulty of making molds

which can be used for such temperatures. 45 The material would also unavoidably receive impurities in casting.

By the method forming my invention it is possible to roll refractory and brittle metals such as tungsten, without danger of 50 cracking. According to the invention the material, if powdered, is then pressed under heavy pressure into a preliminary shape, and is afterward given a cross-section which is similar to the cross-section which the 55 article is to have after it has been rolled, and this is done by a manipulation which causes no changes in the interior of the material to be rolled, but is done by purely external working, such as filing, grinding, 60 planing, cutting and the like. The rolling operation is then begun at about 1000° C. to 1500° C. and the temperature may be gradually lowered during the operation.

What I claim as new and desire to secure 65 by Letters Patent of the United States, is:—

1. The method of preparing refractory metals for rolling free from cracks or fractures which consists in giving to the raw metal prior to rolling and without changing 70 the structure of its internal portions an external shape similar to that of the rolled article and with a transverse section similar to that imposed upon said metal during the 75 rolling operation.

2. The step in the method of rolling refractory metal which consists in externally working the unrolled metal without affecting its internal structure to a shape having 80 a transverse section similar to that assumed by said metal during the operation of rolling.

In witness whereof, I have hereunto set my hand this 5th day of November, 1912.

MARCELLO VON PIRANI.

Witnesses:

HENRY HASPER,  
WOLDEMAR HAUPT.